

No. 784,885.

PATENTED MAR. 14, 1905.

E. L. PRIEST.

METHOD OF EXTRACTING METALS FROM ORE BY ELECTRICITY.

APPLICATION FILED APR. 5, 1904.



Witnesses.

L. J. Allen  
Walter F. Daniel.

Inventor.

Edward L. Priest  
by Frank F. Booth  
his Attorney

## UNITED STATES PATENT OFFICE.

EDWARD L. PRIEST, OF OAKLAND, CALIFORNIA.

## METHOD OF EXTRACTING METALS FROM ORE BY ELECTRICITY.

SPECIFICATION forming part of Letters Patent No. 784,885, dated March 14, 1905.

Application filed April 5, 1904. Serial No. 201,631.

*To all whom it may concern:*

Be it known that I, EDWARD L. PRIEST, a citizen of the United States, residing at Oakland, county of Alameda, State of California, have invented certain new and useful Improvements in Methods of Extracting Metals from Ore by Electricity; and I do hereby declare the following to be a full, clear, and exact description of the same.

10 My invention relates to methods of ore extracting by electricity in which the electric current is closed through the ore and a liquid body by the contact of the two and the formation of an intervening arc, fusing the ore.

15 The difficulty heretofore has been to properly complete the electric current through ore-bodies when the latter are used in any considerable quantity to make the process commercially available.

20 My invention has for its object the utilization of these methods with ore in any quantity; and to this end my invention consists in the novel process or method which I shall hereinafter fully describe.

25 In order to illustrate my method, I refer to the accompanying drawings, in which—

Figure 1 represents a means for carrying out my method in which the ore to be fused is prepared and associated with an electric 30 conductor in one way. Fig. 2 is a similar view showing the ore prepared and associated with the conductor in another shape, but involving the same idea. In this figure the arc-regulator is omitted. Fig. 3 is a similar view 35 illustrating a third way of the same idea.

I prepare the ore by first comminuting it by any suitable means and adding to it or utilizing, if already present, any binding agent which will enable it to remain in or to be 40 pressed into a coherent mass. In some cases water will serve as such agent, or flour or many other pasty or gummy materials may be used. With this coherent comminuted ore mass I associate by incorporation or otherwise, so as to be reduced therewith, a conductor 45 of electricity, which passes through or permeates the mass or otherwise lies in intimate contact with it. This conductor in its best form is carbon in any shape, such as 50 coke or prepared carbon, which serves the

further purpose of a heating medium. The association of this consumable conductor with the comminuted ore mass may be done in various ways. For example, in Fig. 1 I show the ore mass A as having the conductor B passing through its axis. In Fig. 2 I show the conductor B encircling the ore mass A, and in Fig. 3 I show the conductor B incorporated throughout the ore mass A. These will serve to illustrate many forms of association, all of 60 which are rendered possible and practicable by the previous reduction of the ore to a comminuted coherent mass.

In the several figures C is a tank containing a body of liquid, (represented by D,) which 65 liquid may be of any suitable conducting character, such as acidulated or salted water. With this liquid, as by means of the zinc plate d or otherwise, one of the wires, d', of the electric circuit is connected. The other wire, d'', 70 is connected with the conductor B of Figs. 1 and 2 and with a through-wire d<sup>3</sup> in Fig. 3, which wire forms a connection for all the conductor material of that form of ore presentation. Where the prepared-ore masses touch 75 the water, the current is completed through them, and as the arc is established the conductor is consumed, while the ore is reduced and drops into the water. The carbon conductors, as before stated, serve also to heat the ore. 80 These ore masses, with their consumable conductors, may be prepared in any suitable manner, sizes, and numbers, and a plurality of them may be connected in multiple arc. By such initial preparation of the ore the electric 85 current is completed through them and large quantities may be handled with practicability. The metal cannot volatilize as it is precipitated into the water, which also purifies the metal, divesting it of sulfur, the latter forming sulfureted hydrogen, which passes off.

Having thus described my invention, what I claim as new, and desire to secure by Letters Patent, is—

1. The method of extracting metals from 95 ores by electricity, consisting in forming a body of comminuted ore into a coherent mass, associating an electric conductor with the same, and positioning the mass with its conductor in contact with a liquid electrode and 100

passing an electric current through the same to form an arc therebetween.

2. The method of extracting metals from ores by electricity, consisting in first preparing a reducible body comprising a comminuted coherent ore mass and a consumable electric conductor capable of reducing the same, and second in reducing said body by establishing and maintaining an electric arc between said body and a liquid electrode.

3. The method of extracting metals from ores by electricity consisting in preparing a

reducible comminuted coherent ore mass, second, connecting with said mass a consumable electric conductor, and third, contacting said body with a liquid electrode, thereby creating an electric arc therebetween to reduce said body and consume said conductor. 15

In witness whereof I have hereunto set my hand.

EDWARD L. PRIEST.

Witnesses:

WALTER F. VANE,  
D. B. RICHARDS.